

## 1

3,388,445

**METHOD OF MAKING CREASE- AND WRINKLE-RESISTANT FABRICS**

Corrado Mazzolini and Francesco Denti, Mestre, Venezia, Italy, assignors to A.C.S.A. Appliazioni Chimiche S.p.A., Milan, Italy, a corporation of Italy

No Drawing. Filed June 12, 1964, Ser. No. 374,803  
Claims priority, application Italy, June 20, 1963,

12,746/63  
4 Claims. (Cl. 28—76)

**ABSTRACT OF THE DISCLOSURE**

A method of making crease- and wrinkle-resistant fabrics in which fibers are spun from polyvinyl chloride of a high syndiotactic index as produced by polymerization at temperatures from  $-10^{\circ}$  C. to  $-60^{\circ}$  C. and are then twisted into yarns and woven into fabric alone or with a minor proportion of yarn of some other fiber (e. g., wool), the woven fabric being then stretched and subjected to temperatures of  $110^{\circ}$  C. to  $140^{\circ}$  C. for 10 seconds to 30 minutes (preferably  $130^{\circ}$  C. to  $135^{\circ}$  C. for 1 to 10 minutes).

The present invention relates to a process for obtaining crease- and wrinkle-resistant fabrics from textiles based on polyvinyl fibers.

In a preferred form, the present invention relates to a process for obtaining crease- and wrinkle-resistant fabrics from textiles completely or partially made from polyvinyl chloride fibers having a high index of syndiotacticity (IS), achieved by polymerization at a temperature comprised between about  $-10^{\circ}$  C. and about  $-60^{\circ}$  C. in the presence of suitable catalyst acting at such low temperatures. The product so obtained may be spun according to the process claimed in commonly assigned applications Ser. No. 269,257 and No. 310,992.

The invention consists in a process for obtaining a crease- and wrinkle-resistant fabric comprising fibers of a vinyl polymer or predominantly vinylic copolymer in which the fabric is held under tension and maintained at an elevated temperature.

Preferably the fabric comprises polyvinyl chloride or a copolymer which predominantly contains vinyl chloride monomer units, and in a specially preferred form as indicated above, the fabric comprises polyvinyl chloride of a high syndiotactic index obtained by catalysed low temperature polymerization between  $-10^{\circ}$  C. and  $-60^{\circ}$  C.

The fabric may comprise polyvinyl chloride fibers and other synthetic or natural fibers, such as woolen fibers.

The process may be carried out either under dry or humid conditions.

The treatment may be a continuous one (such as for instance in devices of the tenter-frame type) or an intermittent one.

The temperature used for fabrics made of polyvinyl chloride fibers of a high syndiotactic index may be from about  $110^{\circ}$  C. to about  $140^{\circ}$  C. and preferably from  $130^{\circ}$  C. to  $135^{\circ}$  C. As the higher the temperature the greater the antcrease and antiwrinkle effect on the fabric.

The processing time may be from about 10 seconds to about 30 minutes and are preferably from 1 to 10 minutes.

The heat may be transmitted to the fabric by various different means, such as for instance, hot air, steam, nitrogen, or by radiation under infrared rays or the like.

## 2

The fabrics to be processed according to this invention may be either unbleached or dyed with conventional means.

In order to more clearly illustrate the inventive idea of this invention an example is given herebelow without thereby limiting the scope of the invention itself:

Polyvinyl chloride obtained by polymerization at  $-40^{\circ}$  C., with a high syndiotactic index and an intrinsic viscosity ( $\eta$ ) = 1.4 dl. gr.<sup>-1</sup>, is spun into fibers of 3.5 den./filament. 55% of these fibers, with a cut of 40 mm. and dyed with disperse dyes are woven into a fabric with 45% of woollen yarn dyed in tops with an English number Ne of 64s.

The yarn used for the warp has:

15 A metric number Nm.=2/42,  
A twist  $T_z$ =500 turns/meter, and  
A twist  $T_s$ =520 turns/meter.

The yarn used for the weft has:

20 A metric number Nm.=1/20 and  
A twist  $T_z$ =380 turns meter,  
Weave: cloth type  
Number of filaments: 2810 (without selvedge)  
Reed: 57,5/3

25 Width of loom: 163 cm.  
Number of picks: 1730.

The fabric is subjected to the following dressing treatment:

30 (1) Darning  
(2) Scouring  
(3) Washing  
(4) Centrifugation  
35 (5) Drying at  $90^{\circ}$  C. in a tentering machine  
(6) Humidifying

Subsequently a part of the fabric is sheared, steamed to a free shrinkage and subjected to steam decatising. The other part of the sample fabric is heat set at  $135^{\circ}$  C. for 2 minutes under tension and is then sheared, steamed and decatised. The measuring of the crease- and wrinkle-resistance is carried out following the T.B.L. standard method, that is, 1 cm. x 4 cm. samples are conditioned for 24 hours at room temperature and 94% relative humidity, folded, subjected to a pressure load of 500 gr. and subsequently unloaded the wrinkle-recovery angle being measured after 3 minutes.

The wrinkle recovery angle for the sample heat-set according to the invention turned out to be  $130^{\circ}$  in the warp direction as well as in the weft direction while that the fabric not heat-treated according to the invention had a recovery in warp and in weft of only  $100^{\circ}$ .

We claim:

1. A method of making fabric crease- and wrinkle-resistant, the fabric being composed of spun fibers of polyvinyl chloride, with a high syndiotactic index and obtained by polymerization at a temperature between  $-10^{\circ}$  C. and  $-60^{\circ}$  C., twisted into a yarn consisting predominantly of polyvinyl chloride of high syndiotactic index, and with weft and warp interwoven of said yarn to form said fabric, said method comprising the step of subjecting the woven fabric under tension to a heat treatment at a temperature of  $110^{\circ}$  C. to  $140^{\circ}$  C. for a period of 10 seconds to 30 minutes.

2. The method defined in claim 1 wherein the fabric produced is maintained under tension in a tenter frame for a period of 1 to 10 minutes at a temperature between  $130^{\circ}$  C. and  $135^{\circ}$  C.

3. The method defined in claim 1 wherein said fabric contains a minor proportion of a yarn of a material other than of polyvinyl chloride.

4. The method defined in claim 3 wherein said fabric consists of at least 55% by weight polyvinyl chloride yarn with high syndiotactic index and up to 45% by weight of wool yarn, the intrinsic viscosity of the fibers of the polyvinyl chloride being about  $\eta=1.4$  dl. gr.<sup>-1</sup>, the polyvinyl chloride being formed by polymerization at  $-40^{\circ}$  C., said fabric prior to treatment being subjected to washing, centrifugal extraction and drying.

## References Cited

## UNITED STATES PATENTS

|   |           |        |                        |           |
|---|-----------|--------|------------------------|-----------|
| 5 | 2,313,173 | 3/1943 | Schneider et al. ----- | 38—144    |
|   | 2,591,861 | 4/1952 | Pannali -----          | 264—346   |
|   | 2,984,593 | 5/1961 | Isaksen et al. -----   | 264—231 X |

JAMES A. SEIDLECK, Primary Examiner.

ALEXANDER H. BRODMERKEL, Examiner.

T. MORRIS, Assistant Examiner.

UNITED STATES PATENT OFFICE  
CERTIFICATE OF CORRECTION

Patent No. 3,388,445

Dated June 18, 1968

Inventor(s) Corrado Mazzolini et al.

It is certified that error appears in the above-identified patent and that said Letters Patent are hereby corrected as shown below:

In the heading to the specification, line 5, cancel "A.C.S.A. Appliazioni Chimiche" and insert instead -- Chatillon Societa Anonima Italiana per le Fibre Tessili Artificiali --.

SIGNED AND  
SEALED

**JUL 29 1969**

(SEAL)

Attest:

Edward M. Fletcher, Jr.

Attesting Officer

WILLIAM E. SCHUYLER, JR.  
Commissioner of Patents